



US009637913B2

(12) **United States Patent**  
**Ravnaas**

(10) **Patent No.:** **US 9,637,913 B2**  
(b5) **Date of Patent:** **May 2, 2017**

(54) **ACOUSTIC DAMPING COMPOSITIONS  
HAVING ELASTOMERIC PARTICULATE**

(75) Inventor: **Brian Ravnaas**, West Fargo, ND (US)

(73) Assignee: **SAINT-GOBAIN PERFORMANCE  
PLASTICS CORPORATION**, Solon,  
OH (US)

(\*) Notice: Subject to any disclaimer, the term of this  
patent is extended or adjusted under 35  
U.S.C. 154(b) by 398 days.

(21) Appl. No.: **12/757,743**

(22) Filed: **Apr. 9, 2010**

(65) **Prior Publication Data**

US 2010/0261023 A1 Oct. 14, 2010

**Related U.S. Application Data**

(60) Provisional application No. 61/168,466, filed on Apr.  
10, 2009.

(51) **Int. Cl.**  
**E04B 1/84** (2006.01)  
**E04B 1/86** (2006.01)

(52) **U.S. Cl.**  
CPC ..... **E04B 1/86** (2013.01); **E04B 1/84**  
(2013.01); **E04B 2001/8461** (2013.01); **E04B  
2001/8466** (2013.01); **E04B 2001/8476**  
(2013.01); **Y10T 428/31855** (2015.04); **Y10T  
428/31931** (2015.04)

(58) **Field of Classification Search**

CPC ..... E04B 1/86; E04B 2001/8461; E04B 1/74;  
E04B 1/84; E04B 2001/8466; E04B  
2001/8476; Y10T 428/31855; Y10T  
428/31931; Y10T 2001/8461

USPC ..... 428/327, 323  
See application file for complete search history.

(56)

**References Cited**

**U.S. PATENT DOCUMENTS**

|               |         |                      |           |
|---------------|---------|----------------------|-----------|
| 3,489,242 A   | 1/1970  | Gladding et al.      |           |
| 3,615,961 A   | 10/1971 | Meyer                |           |
| 3,658,635 A * | 4/1972  | Eustice .....        | 428/425.8 |
| 3,770,560 A   | 11/1973 | Elder et al.         |           |
| 3,894,169 A   | 7/1975  | Miller               |           |
| 4,299,639 A   | 11/1981 | Bayer                |           |
| 4,416,790 A   | 11/1983 | Schurmann et al.     |           |
| 5,004,764 A * | 4/1991  | Yamamoto et al. .... | 523/400   |
| 5,102,924 A   | 4/1992  | Williams et al.      |           |
| 5,318,837 A   | 6/1994  | Yoshinaka et al.     |           |
| 5,328,957 A * | 7/1994  | Sorathia et al. .... | 525/123   |
| 5,400,296 A   | 3/1995  | Cushman et al.       |           |

(Continued)

**FOREIGN PATENT DOCUMENTS**

|                    |         |
|--------------------|---------|
| DE 102004016099 A1 | 10/2005 |
| EP 0621931 B1      | 7/1997  |

(Continued)

**OTHER PUBLICATIONS**

“Elastomers,” Obtained Mar. 21, 2015, Polymers International Australia, <http://polymers.com.au/elastomers/>.\*

(Continued)

*Primary Examiner* — Nicholas Kokkinos

(74) *Attorney, Agent, or Firm* — Abel Law Group, LLP;  
Thomas H. Osborn

(57) **ABSTRACT**

An acoustic damping composition includes a urethane component, elastomeric particles, and a binder resin including an addition polymer having a carboxylic functional group. The acoustic damping composition can have a Mode 1 Damping Parameter of at least 0.45. The binder resin can have a glass transition temperature of not greater than -25° C.

**20 Claims, 2 Drawing Sheets**



(56)

## References Cited

## U.S. PATENT DOCUMENTS

|                   |         |                              |    |               |         |
|-------------------|---------|------------------------------|----|---------------|---------|
| 5,691,021 A       | 11/1997 | Kobe                         | JP | H01-204954 A  | 8/1989  |
| 5,695,867 A *     | 12/1997 | Saitoh et al. .... 428/219   | JP | 05-032844 A   | 2/1993  |
| 5,858,521 A       | 1/1999  | Okuda et al.                 | JP | H05-032844 A  | 2/1993  |
| 5,923,002 A       | 7/1999  | McGrath et al.               | JP | H06-073228 A  | 3/1994  |
| 6,006,484 A       | 12/1999 | Geissbuhler                  | JP | 07-090126 A   | 4/1995  |
| 6,022,616 A       | 2/2000  | Wu et al.                    | JP | H07-090126 A  | 4/1995  |
| 6,060,553 A       | 5/2000  | Lenczyk et al.               | JP | H10-141434 A  | 5/1998  |
| 6,077,613 A       | 6/2000  | Gaffigan                     | JP | H11-30566 A   | 2/1999  |
| 6,211,320 B1      | 4/2001  | Dershem et al.               | JP | 2972186 B1    | 11/1999 |
| 6,228,939 B1      | 5/2001  | Wang et al.                  | JP | 2001-040165 A | 2/2001  |
| 6,267,347 B1      | 7/2001  | Ryan et al.                  | JP | 2002-544353 A | 12/2002 |
| 6,319,969 B1      | 11/2001 | Walther et al.               | JP | 2003-244788 A | 8/2003  |
| 6,340,519 B1      | 1/2002  | Tanaka et al.                | JP | 2004-250461 A | 9/2004  |
| 6,498,547 B2      | 12/2002 | Morita                       | JP | 2004-269839 A | 9/2004  |
| 6,528,563 B2      | 3/2003  | Kaiser et al.                | JP | 2005-089017 A | 4/2005  |
| 6,789,645 B1      | 9/2004  | Deblander                    | JP | 2006-152020 A | 6/2006  |
| 6,920,723 B2      | 7/2005  | Downey                       | JP | 2006152020 A  | 6/2006  |
| 7,019,102 B2      | 3/2006  | Schoenfeld et al.            | WO | 2008133460 A  | 6/2008  |
| 7,022,746 B2      | 4/2006  | Lockwood et al.              | WO | 2008-169382 A | 7/2008  |
| 7,025,852 B2      | 4/2006  | Kumakura                     | WO | 2008-174701 A | 7/2008  |
| 7,094,811 B2      | 8/2006  | Nodelman et al.              | WO | 9208856       | 5/1992  |
| 7,181,891 B2      | 2/2007  | Surace et al.                | WO | 9315333 A2    | 8/1993  |
| 7,263,028 B2      | 8/2007  | Thomas et al.                | WO | 9520820       | 8/1995  |
| 7,893,149 B2      | 2/2011  | Hermes et al.                | WO | 9731549       | 9/1997  |
| 7,893,151 B2      | 2/2011  | Johnson et al.               | WO | 9733051       | 9/1997  |
| 8,028,800 B2 *    | 10/2011 | Ravnaas .... 181/286         | WO | 9919398       | 4/1999  |
| 2001/0009393 A1   | 7/2001  | Morita                       | WO | 9924520       | 5/1999  |
| 2001/0018228 A1   | 8/2001  | Kumakura                     | WO | 0048832 A1    | 8/2000  |
| 2002/0004538 A1   | 1/2002  | Kaiser et al.                | WO | 0049085 A1    | 8/2000  |
| 2002/0037381 A1   | 3/2002  | Ohira et al.                 | WO | 0069946       | 11/2000 |
| 2002/0160131 A1   | 10/2002 | Ohira et al.                 | WO | 0109078 A1    | 2/2001  |
| 2003/0207491 A1   | 11/2003 | Kumakura                     | WO | 0116231 A1    | 3/2001  |
| 2004/0082721 A1   | 4/2004  | Miura et al.                 | WO | 0123466 A1    | 4/2001  |
| 2004/0113483 A1   | 6/2004  | Sylvester et al.             | WO | 0139969 A1    | 6/2001  |
| 2005/0094311 A1 * | 5/2005  | Boss et al. .... 360/97.01   | WO | 0144136 A1    | 6/2001  |
| 2005/0126851 A1   | 6/2005  | Ikebe et al.                 | WO | 0220687 A2    | 3/2002  |
| 2006/0003104 A1 * | 1/2006  | Chao et al. .... 427/372.2   | WO | 02061010 A2   | 8/2002  |
| 2006/0052474 A1   | 3/2006  | Czerny                       | WO | 03087252 A1   | 10/2003 |
| 2006/0118355 A1   | 6/2006  | Blomeling et al.             | WO | 2004063268 A1 | 7/2004  |
| 2006/0154078 A1   | 7/2006  | Watanabe et al.              | WO | 2005035679 A2 | 4/2005  |
| 2006/0165977 A1   | 7/2006  | Rehfeld et al.               | WO | 2005100709 A1 | 10/2005 |
| 2006/0173103 A1   | 8/2006  | Schmidt                      | WO | 2005118733 A1 | 12/2005 |
| 2006/0183858 A1   | 8/2006  | Takesada et al.              | WO | 2006032802 A1 | 3/2006  |
| 2006/0214341 A1   | 9/2006  | Sugiura et al.               | WO | 2006092560 A1 | 9/2006  |
| 2007/0012509 A1   | 1/2007  | Shimada et al.               | WO | 2006116440 A2 | 11/2006 |
| 2007/0065668 A1   | 3/2007  | Idei                         | WO | 2006131138 A1 | 12/2006 |
| 2007/0088103 A1   | 4/2007  | Poncet                       | WO | 2007017422 A2 | 2/2007  |
| 2007/0101679 A1   | 5/2007  | Harthcock et al.             | WO | 2007019450 A1 | 2/2007  |
| 2007/0160851 A1   | 7/2007  | Barancyk et al.              | WO | 2007053410 A1 | 5/2007  |
| 2007/0224395 A1 * | 9/2007  | Rowitsch et al. .... 428/143 | WO | 2007054699 A2 | 5/2007  |
| 2008/0001431 A1   | 1/2008  | Thompson et al.              | WO | 2007070771 A1 | 6/2007  |
| 2008/0083497 A1   | 4/2008  | Dublineau et al.             | WO | 2007084318 A2 | 7/2007  |
| 2008/0153969 A1   | 6/2008  | Hermes et al.                | WO | 2007149613 A1 | 12/2007 |
| 2008/0249241 A1   | 10/2008 | Heiliger et al.              | WO | 2008002842 A1 | 1/2008  |
| 2008/0250751 A1   | 10/2008 | Pavan et al.                 | WO | 2008005936 A2 | 1/2008  |
| 2009/0013506 A1   | 1/2009  | Mizuhara et al.              | WO | 2008057664 A2 | 5/2008  |
| 2009/0121174 A1   | 5/2009  | Johnson et al.               | WO | 2008115301 A2 | 9/2008  |
| 2009/0305595 A1   | 12/2009 | Ogawa et al.                 |    |               |         |
| 2009/0325446 A1   | 12/2009 | Hori et al.                  |    |               |         |
| 2010/0230206 A1   | 9/2010  | Tinianov et al.              |    |               |         |

## FOREIGN PATENT DOCUMENTS

|    |              |         |
|----|--------------|---------|
| EP | 0897675 A1   | 2/1999  |
| EP | 0588563 B1   | 3/1999  |
| EP | 0965701 A1   | 12/1999 |
| EP | 1031671 A2   | 8/2000  |
| EP | 0966495 B1   | 7/2002  |
| EP | 1408075 A1   | 4/2004  |
| EP | 1161494 B1   | 4/2005  |
| EP | 1160387 B1   | 9/2005  |
| GB | 970392       | 9/1964  |
| GB | 2136063 A    | 9/1984  |
| JP | S63-193977 A | 8/1988  |
| JP | H01-139634 A | 6/1989  |

## OTHER PUBLICATIONS

"Chapter 16. Polymers. Characteristics, Applications, and Processing." Obtained Mar. 21, 2015, University of Virginia, <http://www.virginia.edu/bohr/mse209/chapter16.htm>.\*

J.R. Herrera-Velarde, R. Zenit, D. Chehata, and B. Mena, "The Flow of Non-Newtonian Fluids Around Bubbles and its Connection to the Jump Discontinuity," Mar. 13, 2003, [http://iusti.polytech.univ-mrs.fr/~gep/doctorants/chehata/publiperso/herrera\\_etal\\_JNNFM\\_2002.pdf](http://iusti.polytech.univ-mrs.fr/~gep/doctorants/chehata/publiperso/herrera_etal_JNNFM_2002.pdf).\*

Zheng, Zhu et al.; "Elastomeric Reactive Microgels as Toughener for Epoxy Adhesives," Chinese Journal of Polymer Science, 1987, vol. 5, pp. 76-80.

Texanol, Case No. 25265-77-4; UNEP Publications; IRPTC Data Profile, Identifiers, Physical and Chemical Properties pp. 73-117.

International Search Report from PCT/U52010/030586 dated Nov. 26, 2010, 1 pg.

International Search Report from PCT/US2010/030587 dated Nov. 26, 2010, 1 pg.

(56)

**References Cited**

OTHER PUBLICATIONS

Wang, Horng-Jou et al, "Vibration and damping analysis of a three-layered composite annular plate with a viscoelastic mid-layer," *Composite Structures*, Dec. 2002, pp. 563-570, vol. 58, No. 4, Elsevier Science Ltd.

\* cited by examiner



**FIG. 3****FIG. 4**

## 1

ACOUSTIC DAMPING COMPOSITIONS  
HAVING ELASTOMERIC PARTICULATECROSS-REFERENCE TO RELATED  
APPLICATION(S)

The present application claims priority from U.S. Provisional Patent Application No. 61/168,466, filed Apr. 10, 2010, entitled "ACOUSTIC DAMPING COMPOSITIONS HAVING ELASTOMERIC PARTICULATE," naming inventor Brian Ravnaas, which application is incorporated by reference herein in its entirety.

## FIELD OF THE DISCLOSURE

This disclosure, in general, relates to acoustic damping compositions, construction materials formed using such acoustic damping compositions, and methods of using acoustic damping compositions.

## BACKGROUND

Noise control has long been an issue in residential and business settings. With increasing urbanization and an increasing cost of real estate, individuals are living and working in closer proximity, increasing the need for noise reduction, particularly in high rise and apartment settings. To combat noise in such urban settings, several cities, states and countries have implemented noise control building codes. Further, many building owners specify noise tolerance in construction specifications during construction.

However, many conventional methods for controlling noise are either cumbersome to install or ineffective. Particularly in the case of walls, conventional techniques include the use of resilient members disposed between a wall panel and a support. Such resilient members can be difficult to install and are expensive. Other conventional methods include the installation of thick insulative members which have limited effectiveness and add additional steps to the installation and construction of walls or ceilings.

Another technique used for controlling noise is the use of a damping material between layers of construction material, such as plywood or drywall. Such damping materials are also referred to as constrained layer damping materials. However, conventional damping materials provide limited sound control for particular noise.

As such, an improved acoustic damping composition would be desirable.

## BRIEF DESCRIPTION OF THE DRAWINGS

The present disclosure may be better understood, and its numerous features and advantages made apparent to those skilled in the art by referencing the accompanying drawings.

FIG. 1 includes and illustration of an exemplary construction panel.

FIG. 2 includes an illustration of an acoustic testing apparatus.

FIG. 3 and FIG. 4 include illustrations of exemplary mounted construction panels.

The use of the same reference symbols in different drawings indicates similar or identical items.

DESCRIPTION OF THE PREFERRED  
EMBODIMENT(S)

In a particular embodiment, an acoustic damping composition includes a binder resin, a modifying resin, and elas-

## 2

tomeric particles. In an example, the binder resin is an addition polymer having a carboxylic functional group. For example, the binder resin may be an acrylic component. The modifying resin may include a urethane component. The elastomeric particles may have an average particle size of not greater than 850 micrometers and may have a modulus of elasticity of not greater than 20 MPa. The acoustic damping composition has a Mode 1 Damping Parameter of at least 0.45. In addition, the acoustic damping composition may have a Mode 2 Damping Parameter of at least 0.27 or a Mode 3 Damping Parameter of at least 0.27. Such an acoustic damping composition may be incorporated into a construction panel, for example, between two rigid panels.

In an example, the acoustic damping composition may be extruded on a first major surface of a first rigid panel. A first major surface of a second rigid panel may be contacted with the acoustic damping composition to form a laminate that may be used in the construction of walls, ceilings, or floors.

In particular, the acoustic damping composition may be formulated as a water-based emulsion including the binder resin, modifying resin, and elastomeric particles. When applied, the water of the water-based emulsion may evaporate to leave the binder resin, the modifying resin, and elastomeric particles of the acoustic damping composition.

In an exemplary embodiment, the binder resin is an addition polymer having a carboxylic functional group, such as a carboxylic acid or an ester derivative functional group. An addition polymer is a polymer formed through addition polymerization as opposed to condensation polymerization.

In an example, the binder resin is formed from a monomer, such as acrylic acid, methyl methacrylate, ethyl methacrylate, methacrylate, methyl acrylate, ethyl acrylate, vinyl acetate, derivatives thereof, or any combination thereof. For example, the binder resin may include polyvinyl acetate, a derivative thereof, or a copolymer thereof. In a further example, the polyvinyl acetate may be modified, such as through hydroxylization to form a copolymer poly(vinyl acetate-co-vinyl alcohol).

In another example, the binder resin may be an acrylic resin. The acrylic resin may have an alkyl group having from 1-4 carbon atoms, a glycidyl group or a hydroxyalkyl group having from 1-4 carbon atoms. Representative acrylic polymers include polyacrylate, polymethyl methacrylate, polyethyl methacrylate, polybutyl methacrylate, polyglycidyl methacrylate, polyhydroxyethyl methacrylate, polymethyl acrylate, polyethyl acrylate, polybutyl acrylate, polyglycidyl acrylate, polyhydroxyethyl acrylate, or any combination thereof. In a particular example, the acrylic resin is in the form of an emulsion, such as a water-based emulsion. For example, the acrylic resin may be an adhesive acrylic resin, such as a pressure-sensitive adhesive acrylic resin.

In particular, the binder resin has a low glass transition temperature. For example, the glass transition temperature of the binder resin may be not greater than -25° C. In an example, the glass transition temperature is not greater than -40° C., such as not greater than -50° C. Further, the glass transition temperature of the binder resin may be not greater than -60° C.

In addition, the binder resin may have a molecular weight of at least 8,000 atomic units, such as at least 10,000 atomic units, at least 20,000 atomic units, or even as high as 25,000 atomic units or higher. In particular, the average molecular weight of the binder resin is not greater than 100,000 atomic units.

In a particular embodiment, the binder resin is a viscoelastic resin, exhibiting a hysteresis on a stress versus strain graph.

Further, the acoustic damping composition includes a modifying resin. The modifying resin may be an acrylic resin, a urethane resin, an epoxy resin, an acrylate/amine resin, or any combination thereof. In general, the modifying resin is self-dispersible in aqueous emulsions and is immiscible with the binder resin.

In a particular embodiment, the modifying resin is a urethane resin formed from reactants including isocyanate, an ether alcohol, and an ester alcohol. In a particular embodiment, the isocyanate component includes a diisocyanate monomer. An exemplary diisocyanate monomer may include toluene diisocyanate, m-phenylene diisocyanate, p-phenylene diisocyanate, xylene diisocyanate, 4,4'-diphenylmethane diisocyanate, hexamethylene diisocyanate, isophorone diisocyanate, polymethylene polyphenyl diisocyanate, 3,3'-dimethyl-4,4'-biphenylene diisocyanate, 3,3'-dimethyl-4,4'-diphenylmethane diisocyanate, 3,3'-dichloro-4,4'-biphenylene diisocyanate, or 1,5-naphthalene diisocyanate; their modified products, for instance, carbodiimide-modified products; or the like, or any combination thereof. Such diisocyanate monomers may be used alone or in admixture of at least two kinds. In a particular example, the isocyanate component may include methylene diphenyl diisocyanate (MDI), toluene diisocyanate (TDI), hexamethylene diisocyanate (HDI), isophorone diisocyanate (IPDI), or any combination thereof. In an example, the isocyanate may include methylene diphenyl diisocyanate (MDI) or toluene diisocyanate (TDI). In particular, the isocyanate includes methylene diphenyl diisocyanate (MDI).

In an example, the isocyanate forms 10 wt % to 50 wt % of the reactants that form the urethane component. For example, the isocyanate may form 20 wt % to 40 wt % of the reactants, such as 25 wt % to 35 wt % of the reactants.

In an example, the ether alcohol may include a polyether polyol or an alkoxy derivative thereof. A suitable polyether polyol useful for production of the modifying resin can be produced by polyinsertion via double metal cyanide (DMC) catalysis of alkylene oxides, by anionic polymerization of alkylene oxides in the presence of alkali hydroxides or alkali alcoholates as catalysts and with the addition of at least one initiator molecule containing 2 to 6, preferably 2 to 4, reactive hydrogen atoms in bonded form, or by cationic polymerization of alkylene oxides in the presence of Lewis acids, such as antimony pentachloride or boron fluoride etherate. A suitable alkylene oxide may contain 2 to 4 carbon atoms in the alkylene radical. An example includes tetrahydrofuran, 1,2-propylene oxide, 1,2- or 2,3-butylene oxide; ethylene oxide, 1,2-propylene oxide, or any combination thereof. The alkylene oxides can be used individually, in succession, or as a mixture. In particular, mixtures of 1,2-propylene oxide and ethylene oxide may be used, whereby the ethylene oxide is used in quantities of 10% to 50% as an ethylene oxide terminal block so that the resulting polyols display over 70% primary OH terminal groups. An example of an initiator molecule includes water or dihydric or trihydric alcohols, such as ethylene glycol, 1,2-propanediol and 1,3-propanediol, diethylene glycol, dipropylene glycol, ethane-1,4-diol, glycerol, trimethylol propane, or any combination thereof.

Suitable polyether polyols, such as polyoxypropylene polyoxyethylene polyols, have average functionalities of 1.6 to 2.4, such as 1.8 to 2.4, and number-average molecular weights of 800 g/mol to 25,000 g/mol, such as 800 g/mol to 14,000 g/mol, particularly 2,000 g/mol to 9,000 g/mol. Difunctional or trifunctional polyether polyols having a number-average molecular weight of 800 g/mol to 25,000

g/mol, such as 800 g/mol to 14,000 g/mol, or even 2,000 g/mol to 9,000 g/mol, may be used as polyol components.

In a particular example, the polyether polyol includes polyethylene glycol, methoxy derivatives thereof, ethoxy derivatives thereof, or any combination thereof. The polyethylene glycol or derivative thereof may include between 3 and 20 ethylene glycol units, such as between 5 and 20 ethylene glycol units, or even between 5 and 15 ethylene glycol units. Further, the ether alcohol may include blends of 10 polyethylene glycol or derivatives thereof having a different number of ethylene glycol units. Another exemplary ether alcohol includes phenyl alcohol-based glycol ethers.

In another example, the ether alcohol component may include a polypropylene glycol alkyl ether. In an example, 15 the polypropylene glycol alkyl ether may include dipropylene glycol n-butyl ether, tripropylene glycol n-butyl ether, or any combination thereof.

In a particular embodiment, the reactants that form the polyurethane include at least 15% by weight of the dipropylene glycol n-butyl ether. For example, the reactants may include at least 20% by weight of the dipropylene glycol n-butyl ether, such as at least 25% by weight of the dipropylene glycol n-butyl ether. In particular, the reactants may include not greater than 50% by weight of the dipropylene glycol n-butyl ether. Further, the reactants may include tripropylene glycol n-butyl ether in an amount in a range of 0% to 30% by weight, such as a range of 5% to 20% by weight, or even a range of 10% to 20% by weight. When the reactants that form the polyurethane include both dipropylene glycol n-butyl ether and tripropylene glycol n-butyl ether, the components may be included in a ratio (dipropylene glycol n-butyl ether/tripropylene glycol n-butyl ether) of at least 0.5, such as at least 1.0, or even at least 1.5. Alternatively, the reactants may include tripropylene glycol n-butyl ether as the only polypropylene glycol alkyl ether.

In addition, the reactants of the urethane resin may include an ester alcohol. For example, the ester alcohol may be a polyester polyol. In an exemplary embodiment, a polyester polyol is derived from dibasic acids such as adipic, 40 glutaric, fumaric, succinic or maleic acid, or anhydrides and di-functional alcohols, such as ethylene glycol, diethylene glycol, propylene glycol, di or tripropylene glycol, 1-4 butane diol, 1-6 hexane diol, or any combination. For example, the polyester polyol may be formed by the condensation reaction of the glycol and the acid with the continuous removal of the water by-product. A small amount of high functional alcohol, such as glycerin, trimethanol propane, pentaerythritol, sucrose or sorbitol or polysaccharides may be used to increase branching of the polyester polyol. The esters of simple alcohol and the acid may be used via an ester interchange reaction where the simple alcohols are removed continuously like the water and replaced by one or more of the glycols above. Additionally, polyester polyols may be produced from aromatic acids, 50 such as terephthalic acid, phthalic acid, 1,3,5-benzoic acid, their anhydrides, such as phthalic anhydride.

In a particular example, the ester alcohol may include an alkyl diol alkyl ester. For example, the alkyl diol alkyl ester may include trimethyl pentanediol isobutyrate, such as 2,2, 60 4-trimethyl-1,3-pentanediol isobutyrate. In particular, desirable acoustic damping is observed when the ester alcohol includes trimethyl pentanediol isobutyrate and the ether alcohol includes dipropylene glycol n-butyl ether. Alternatively, advantages are exhibited when the ester alcohol includes trimethyl pentanediol isobutyrate and the ether alcohol includes dipropylene glycol n-butyl ether and tripropylene glycol n-butyl ether. In an exemplary embodiment,

the reactants may include the ester alcohol, such as the alkyl diol alkyl ester, in a range of 1.0 wt % to 8.0 wt %, such as a range of 2.0 wt % to 6.0 wt %.

In a particular embodiment, the acoustic damping composition includes a binder resin and modifying resin that are immiscible. For example, the binder resin and modifying resin form separate phases when dried as a film. In particular, the acoustic damping composition may have a haze value as measured by ASTM D1003 (method B) of at least 30%, such as at least 50%.

In the acoustic damping composition, the binder resin and modifying resin may be included in a ratio (binder resin/modifying resin) in a range between 0.5 and 1.5. For example, the range may be between 0.8 and 1.3. In particular, the binder resin is an acrylic component and the modifying resin is a urethane component. As such, the ratio of acrylic component to urethane component is in a range between 0.5 and 1.5, such as a range between 0.8 and 1.3.

In addition, the acoustic damping composition may include elastomeric particles. In an example, the elastomeric particles may include a polyolefin rubber, a diene elastomer, a silicone rubber, or any combination thereof. For example, the polyolefin may include a homopolymer, a copolymer, a terpolymer, an alloy, or any combination thereof formed from a monomer, such as ethylene, propylene, butene, pentene, methyl pentene, octene, or any combination thereof. An exemplary polyolefin includes polyethylene, ethylene propylene copolymer, ethylene butene copolymer, polypropylene (PP), polybutylene, polypentene, polymethylpentene, polystyrene, ethylene octene copolymer, or any combination thereof. In particular, the polyolefin rubber may include polybutylene.

In another example, the elastomeric particles may include a diene elastomer. In an exemplary embodiment, the diene elastomer is a copolymer formed from at least one diene monomer. For example, the diene elastomer may be a copolymer of ethylene, propylene and diene monomer (EPDM). An exemplary diene monomer includes a conjugated diene, such as butadiene, isoprene, chloroprene, or the like; a non-conjugated diene including from 5 to about 25 carbon atoms, such as 1,4-pentadiene, 1,4-hexadiene, 1,5-hexadiene, 2,5-dimethyl-1,5-hexadiene, 1,4-octadiene, or the like; a cyclic diene, such as cyclopentadiene, cyclohexadiene, cyclooctadiene, dicyclopentadiene, or the like; a vinyl cyclic ene, such as 1-vinyl-1-cyclopentene, 1-vinyl-1-cyclohexene, or the like; an alkylbicyclononadiene, such as 3-methylbicyclo-(4,2,1)-nona-3,7-diene, or the like; an indene, such as methyl tetrahydroindene, or the like; an alkenyl norbornene, such as 5-ethylidene-2-norbornene, 5-butylidene-2-norbornene, 2-methylallyl-5-norbornene, 2-isopropenyl-5-norbornene, 5-(1,5-hexadienyl)-2-norbornene, 5-(3,7-octadienyl)-2-norbornene, or the like; a tricyclodiene, such as 3-methyltricyclo (5,2,1,0.sup.2,6)-deca-3,8-diene or the like; or any combination thereof. In a particular embodiment, the diene includes a non-conjugated diene. In another embodiment, the diene elastomer includes alkenyl norbornene. The diene elastomer may include, for example, ethylene from about 63 wt % to about 95 wt % of the polymer, propylene from about 5 wt % to about 37 wt %, and the diene monomer from about 0.2 wt % to about 15 wt %, based upon the total weight of the diene elastomer. In a particular example, the ethylene content is from about 70 wt % to about 90 wt %, propylene from about 17 wt % to about 31 wt %, and the diene monomer from about 2 wt % to about 10 wt % of the diene elastomer. In general, the diene elastomer includes a small amount of a diene monomer, such as a dicyclopentadiene, a ethylnorbornene, a methylnor-

bornene, a non-conjugated hexadiene, or the like, and typically has a number average molecular weight of from about 50,000 to about 100,000. Exemplary diene elastomers are commercially available under the tradename NORDEL from Dow, such as NORDEL IP 4725P. In a particular example, the elastomeric material includes a blend of a diene elastomer and a polyolefin.

In another example, the elastomeric particles may include a silicone elastomer, such as a polyalkylsiloxane, a phenyl silicone, a fluorosilicone, or any combination thereof. For example, the silicone polymer may, for example, include polyalkylsiloxanes, such as silicone polymers formed of a precursor, such as dimethylsiloxane, diethylsiloxane, dipropylsiloxane, methylmethysiloxane, methylpropylsiloxane, or any combination thereof. In a particular embodiment, the polyalkylsiloxane includes a polydialkylsiloxane, such as polydimethylsiloxane (PDMS).

In particular, the elastomeric particles form a separate phase from the binder resin and modifying resin. The separate phase takes the form of distinct particles. For example, the elastomeric particles may have an average size of not greater than 850 micrometers. In an example, the average particle size is not greater than 600 micrometers, such as not greater than 450 micrometers, or even not greater than 250 micrometers. In a particular example, the average particle size is at least 1 micrometer, such as at least 10 micrometers.

The elastomeric particles may be formed of a material having a desirable modulus of elasticity. In an example, the elastomeric particles may be formed of a material having a modulus of elasticity of not greater than 20 MPa. For example, the modulus of elasticity may be in a range of 0.1 MPa to 20 MPa, such as a range of 0.1 MPa to 10 MPa.

In a particular example, the acoustic damping composition may include the elastomeric particles in an amount of 0.1 wt % to 50 wt %. For example, the acoustic damping composition may include the elastomeric particles in an amount of 0.1 wt % to 25 wt %, such as an amount of 3 wt % to 12 wt %.

In a further exemplary embodiment, the acoustic damping composition may include a second set of elastomeric particles. For example, the second set of elastomeric particles may have an average particle size of at least 580 micrometers, such as at least 840 micrometers. In particular, the average particle size of the second elastomeric particles may be greater than the first elastomeric particles. The second elastomeric particles may be included in the acoustic damping composition in amounts of 0.1 wt % to 7 wt %, such as amounts of 0.5 wt % to 5 wt %. The composition of the second elastomeric particles may be selected from the compositions disclosed above in relation to the first elastomeric particles. In particular, the second elastomeric particles may have a composition similar to the first elastomeric particles. Alternatively, the composition of the second elastomeric particles may be different than the composition of the first elastomeric particles.

In an exemplary embodiment, the acoustic damping composition may be prepared as a water-based emulsion including the binder resin, the modifying resin, and the elastomeric particles. In an example, the solids content of the water-based emulsion, including the binder resin and modifying resin, is at least 40%. For example, the solids content of the water-based emulsion may be at least 50%, such as least 60%, or even at least 65%. In addition, the water-based emulsion may have a desirable pH. For example, the pH may be in a range of 6.8 to 8.0, such as in a range of 7.0 to 7.5.

Further, the water-based emulsion may have a viscosity in a range of 1,000 cps to 500,000 cps. For example, the viscosity may be in a range of 1,000 cps to 100,000 cps, such as a range of 5,000 cps to 50,000 cps, as measured with a #6 spindle at 10 rpm. In particular, the viscosity may be in a range of 10,000 cps to 40,000 cps, such as a range of 20,000 cps to 35,000 cps. To control the viscosity, a thickening agent may be added to the water-based emulsion. For example, the thickener may be an anionic thickener or a nonionic thickener. In a further example, the thickener may be a cellulose-based or modified cellulose-based thickener, an associative thickener, an inverse emulsion thickener, or an alkali swellable emulsion thickener. Compositionally, the thickener may include polyacrylate or polymethacrylate, carboxylate, polyvinyl alcohol, polyacrylamide, or any combination thereof. In a particular example, the thickener includes an acrylate thickener. Further, the thickener may have an average molecular weight in a range of 30,000 to 70,000 atomic units, such as a range of 40,000 to 55,000 atomic units. The thickener may be included in an amount 0.1 wt % to 5 wt %.

Once deployed and dried, the acoustic damping composition exhibits desirable acoustic damping, such as a desirable Mode 1 Damping Parameter, a Mode 2 Damping Parameter, or a Mode 3 Damping Parameter. The Mode 1 Damping Parameter, Mode 2 Damping Parameter, and Mode 3 Damping Parameter are defined below in relation to the specified testing method of the Examples. In an example, the acoustic damping composition may have a Mode 1 Damping Parameter of at least 0.45. For example, the Mode 1 Damping Parameter may be at least 0.5, such as at least 0.55, at least 0.6, at least 0.65, or even at least 0.7. Further, the acoustic damping composition may have a Mode 2 Damping Parameter of at least 0.27, such as at least 0.30, or even at least 0.32. In addition, the acoustic damping composition may have a Mode 3 Damping Parameter of at least 0.27, such as at least 0.31.

In a further example, the acoustic damping composition may exhibit a desirable Damping Performance, defined as the percent increase in mode Damping Parameter determined in accordance with the testing method specified in the Examples relative to the noiseproofing compound that is commercially available under the tradename GREEN GLUE in August 2008 from The Green Glue Company of West Fargo, N. Dak. For example, the acoustic damping composition may have a Mode 1 Damping Performance of at least 20%, such as at least 30%, at least 40%, at least 50% or even at least 60%. In another example, the acoustic damping composition may have a Mode 2 Damping Performance of at least 20%, such as at least 30%, at least 40%, or even at least 50%. In an additional example, the acoustic damping composition may have a Mode 3 Damping Performance of at least 10%.

In addition, the acoustic damping composition may include a ceramic particulate having an average particle size of not greater than 100 micrometers. For example, the acoustic damping composition may include not greater than 50 wt % of the ceramic particulate, such as between 2 wt % and 25 wt % of the ceramic particulate. In an example, the ceramic particulate has an average particle size of not greater than 50 micrometers, such as not greater than 25 micrometers, or even not greater than 10 micrometers. In a particular example, the average particle size of the ceramic particulate may be less than 1 micrometer, such as less than 100 nanometers. For example, the ceramic particulate may include an aluminous ceramic, such as alumina trihydrate. In

another example, the ceramic particulate may include silica, zirconia, titania, alumina, or any combination thereof.

In use, the acoustic damping composition may be disposed between two relatively flat rigid members. For example, the acoustic damping composition may be laminated between two rigid panels to form a construction panel for use in forming walls, ceilings, or floors. For example, the rigid panels may include wood, plywood, gypsum board, cement board, plaster board, wallboard, gyproc, sheetrock, or any combination thereof. In an example, the acoustic damping composition may be used to form a laminate for manufacturing walls. In another example, the acoustic damping composition may be disposed between subflooring and flooring. In a further example, the acoustic damping composition may be disposed between rigid members of a ceiling panel.

For example, as illustrated in FIG. 1, a construction panel 100 includes an acoustic damping composition layer 102 disposed between a first rigid panel member 104 and a second rigid panel member 106. In particular, when disposed between the two rigid panels (104 and 106), the acoustic damping composition may have a thickness in a range of 25 micrometers to 5 millimeters, such as a range of 100 micrometers to 5 millimeters, a range of 500 micrometers to 5 millimeters, or even a range of 1 millimeter to 5 millimeters. Alternatively, or in addition, an additional layer (not illustrated) of acoustic damping composition may be applied to the second major surface of the rigid panel 106. Another rigid panel (not illustrated) may be applied in contact with the second layer of acoustic damping composition to form a three rigid member panel with two acoustic composition layers.

In particular, preformed laminates may be formed using the acoustic damping composition. For example, the acoustic damping composition may be applied to a surface of a first rigid panel. The surface of the second rigid panel is placed in contact with the acoustic damping composition that is in contact with a major surface with the first rigid panel to form the laminate.

Particular embodiments of the above described acoustic damping composition exhibit technical advantages. In particular, embodiments of the above described exhibit desirable damping of Mode 1, Mode 2 and Mode 3 vibrations. In addition, embodiments of the acoustic damping composition enhance acoustic damping, particularly after installation.

As illustrated in FIG. 3, when a construction panel 300 is attached to a support structure 310, portions of the construction panel 300 deform around the attachment point. In an example, the construction panel 300 includes an acoustic damping layer 302 disposed between an outer member 304 and an inner member 306. When the construction panel 300 is attached to a support 310 using a nail or screw 308, the outer member 304 and the acoustic damping layer 302 deform, to form a pinch point. Excess deformation can cause the outer member 304 to contact the inner member 306, circumventing the acoustic damping provided by the acoustic damping layer 302. When elastomeric particles 312 are disposed in the acoustic damping layer 302, the potential for contact between the outer member 304 and the inner member 306 may be limited, maintaining improved acoustic damping. In particular, the elastomeric particles are not viscous and lodge between the inner member 306 and the outer member 304 at pinch points, providing for some damping at pinch points. In contrast, FIG. 4 illustrates portions of a construction panel 400 in which a nail or screw 408 causes excess deformation. Absent elastomeric particles, the acoustic damping layer 402 deforms, allowing the

outer and inner members 404 and 406 to contact, providing a path for easy transmission of sound.

### EXAMPLES

Each of the acoustic damping compositions described below are tested for damping of Mode 1, Mode 2, and Mode 3 vibrations. In particular, the test procedure is described below. The output of the procedure provides Damping Parameters for Mode 1, Mode 2, and Mode 3 vibrations, respectively defined as the Mode 1 Damping Parameter, the Mode 2 Damping Parameter, and the Mode 3 Damping Parameter. As defined herein, Mode 1 is the fundamental mode of the long dimension of the test panel, Mode 2 is the 2nd order mode of the long dimension of the test panel, and Mode 3 is the fundamental mode of the narrow dimension of the panel.

To test the formulations, each formulation is applied between two layers of  $\frac{1}{2}$  inch thick drywall having dimensions 8"×24" to form a panel. The formulations are applied using a  $\frac{3}{16}$  inch plastic V notch trowel. The panels are dried for approximately 30 days.

To test the panels, an acoustic testing apparatus 200 includes the panel 202 placed on a 2-inch thick pad of low density/low modulus open cell polyurethane acoustic foam 204 having a density of approximately 1.7 lb/cuft, as illus-

5 factors of at least three selected responses are arithmetically averaged to yield a damping parameter. The Mode 1 Damping Parameter is the damping parameter for Mode 1. The Mode 2 Damping Parameter is the damping parameter for Mode 2. The Mode 3 Damping Parameter is the damping parameter for Mode 3.

10 While the low density/low modulus open cell polyurethane foam may contribute to some damping, the damping contribution of the foam is not more than 0.01 and as such, is determined to be low enough to not affect the results of the experiments below.

15

### Example 1

20 Formulations are prepared from water-based emulsions having a 62% solids content. Each formulation includes 100 parts binder resin (FLEXACRYL AF-2027, available from Air Products), 90 parts of a modifying resin described in Table 1, and 45 parts water. Each formulation is thickened to approximately 30,000 cps as measured with a #6 spindle at 10 rpm. The viscosity is adjusted using TEXIPOL 237, available from Scott Bader, UK. Ammonia is used to raise the pH to between 7 and 7.5.

TABLE 1

| Component    | Sample Compositions |     |     |     |     |     |     |     |     |
|--------------|---------------------|-----|-----|-----|-----|-----|-----|-----|-----|
|              | #1                  | #2  | #3  | #4  | #5  | #6  | #7  | #8  | #9  |
| TPnB         | 240                 | 120 | 0   | 145 | 176 | 176 | 360 | 400 | 240 |
| DPnB         | 240                 | 240 | 360 | 288 | 176 | 176 | 0   | 0   | 120 |
| Texanol      | 0                   | 40  | 40  | 0   | 40  | 20  | 40  | 0   | 40  |
| CARBOWAX 550 | 91                  | 78  | 80  | 86  | 75  | 72  | 76  | 76  | 80  |
| MDI          | 319                 | 278 | 296 | 301 | 261 | 248 | 238 | 238 | 258 |

Numbers represent grams of component

TPnB—tripropylene glycol n-butyl ether

DPnB—dipropylene glycol n-butyl ether

Texanol—trimethyl pentanediol isobutyrate, available from Eastman Chemical Company

CARBOWAX 550—methoxy terminated polyethylene glycol available from Dow Chemical Company

MDI—methylene diphenyl diisocyanate

TABLE 2

|        | Mode Frequencies for Sample Compositions |        |         |        |        |        |        |        |        |
|--------|------------------------------------------|--------|---------|--------|--------|--------|--------|--------|--------|
|        | Mode Frequency (Hz)                      |        |         |        |        |        |        |        |        |
|        | #1                                       | #2     | #3      | #4     | #5     | #6     | #7     | #8     | #9     |
| Mode 1 | 123.67                                   | 123.33 | 135.33  | 129.00 | 125.00 | 124.00 | 121.00 | 116.67 | 124.50 |
| Mode 2 | 432.67                                   | 429.67 | 473.67  | 448.00 | 428.00 | 424.00 | 418.00 | 421.67 | 425.33 |
| Mode 3 | 981.67                                   | 956.33 | 1006.33 | 974.00 | 945.33 | 945.33 | 929.67 | 947.00 | 947.33 |

55

TABLE 3

|        | Mode Damping Parameters for Sample Compositions |      |      |      |      |      |      |      |      |
|--------|-------------------------------------------------|------|------|------|------|------|------|------|------|
|        | Mode Damping Parameter                          |      |      |      |      |      |      |      |      |
|        | #1                                              | #2   | #3   | #4   | #5   | #6   | #7   | #8   | #9   |
| Mode 1 | 0.61                                            | 0.76 | 0.62 | 0.67 | 0.75 | 0.69 | 0.70 | 0.58 | 0.70 |
| Mode 2 | 0.35                                            | 0.34 | 0.39 | 0.36 | 0.32 | 0.33 | 0.30 | 0.31 | 0.34 |
| Mode 3 | 0.30                                            | 0.30 | 0.34 | 0.31 | 0.30 | 0.30 | 0.27 | 0.27 | 0.29 |

60

trated in FIG. 2. An accelerometer 206 (Measurement Specialties ACH-01 piezoelectric accelerometer or equivalent having a resonant frequency significantly greater than the frequency range 20 Hz-500 Hz) is placed in the center of the panel. The panel is struck a total of at least 12 times and the resulting impulses are recorded and saved. Three of the twelve impulses are selected at random and analyzed. The impulse response is analyzed using a fast Fourier transform techniques to identify three modes of vibration using a fast Fourier transform software or a system, such as a Brüel & Kjaer Pulse system. A three decibel rule is applied to determine the damping factor. For each mode, the damping

65

Table 2 illustrates the mode frequencies for each sample, and Table 3 illustrates the damping parameter for each sample. The Texanol component provides improvement in Mode 1 damping. In particular, those samples including Texanol exhibit an average Mode 1 Damping Parameter of 0.7, while those samples without Texanol exhibit an average Mode 1 Damping Parameter of 0.62. In addition, the presence of DPnB provides some advantages, as does the combination of DPnB with TPnB. For example, formulas with the combination of DPnB and TPnB exhibit an average Mode 1 damping of 0.7 compared to an average Mode 1 damping of 0.63 without the combination. Further, the presence of DPnB correlates well with Mode 2 damping. Furthermore, the combination of DPnB, TPnB and Texanol provides an average Mode 1 Damping Parameter of 0.73, while formulas not having this entire combination average 0.64.

#### Example 2

Three samples are prepared having different solids content. The formulations are thickened with TEXIPOL 253, available from Scott Bader, UK. Table 4 illustrates the resonance frequencies for the Modes 1, 2 and 3.

TABLE 4

| Mode Frequencies for Sample Compositions |            |            |
|------------------------------------------|------------|------------|
| Mode Frequency (Hz)                      |            |            |
| 58% solids                               | 65% solids | 72% solids |
| Mode 1                                   | 122.00     | 116.00     |
| Mode 2                                   | 422.00     | 399.00     |
| Mode 3                                   | 920.00     | 908.00     |

As the solid content increases, the location of the resonance modes appears to drop in frequency, implying a softer damping film. Such an effect may also reflect changes in the thickness of the damping film. While the same trowel is used for each sample, the higher solids samples have slightly thicker films. Thicker films tend to translate to softer film, all things being equal.

TABLE 5

| Mode Damping for Sample Compositions |            |            |
|--------------------------------------|------------|------------|
| Mode Damping                         |            |            |
| 58% solids                           | 65% solids | 72% solids |
| Mode 1                               | 0.64       | 0.70       |
| Mode 2                               | 0.39       | 0.34       |
| Mode 3                               | 0.33       | 0.36       |

Table 5 illustrates the effect of damping for each of the modes. As illustrated, the Mode 1 Damping Parameter increases with increasing solids content. However, Mode 3 damping appears to decrease with increasing solids content while the Mode 3 Damping Parameter undergoes a maximum around 65% solids.

#### Example 3

Samples are prepared using different thickeners. In particular, samples are prepared using TEXIPOL 253, TEXIPOL 237, and TEXIPOL 258, available from Scott Bader, UK. The samples are prepared in accordance with Sample 3 of Example 1.

TABLE 6

| 5      | Mode Frequencies for Sample Compositions |             |             |
|--------|------------------------------------------|-------------|-------------|
|        | Mode Frequency (Hz)                      |             |             |
|        | TEXIPOL 253                              | TEXIPOL 237 | TEXIPOL 258 |
| Mode 1 | 120                                      | 122         | 121         |
| Mode 2 | 422                                      | 442         | 417         |
| Mode 3 | 920                                      | 965         | 914         |

TABLE 7

| 15     | Mode Damping for Sample Compositions |             |             |
|--------|--------------------------------------|-------------|-------------|
|        | Mode Damping                         |             |             |
|        | TEXIPOL 253                          | TEXIPOL 237 | TEXIPOL 258 |
| Mode 1 | 0.64                                 | 0.53        | 0.54        |
| Mode 2 | 0.39                                 | 0.42        | 0.40        |
| Mode 3 | 0.33                                 | 0.36        | 0.35        |

As illustrated in Table 6, only slight differences are exhibited in the resonance frequencies of the modes. As illustrated in Table 7, the thickener provides a large change in damping parameter, particularly the Mode 1 Damping Parameter.

#### Example 4

30 Commercially available acoustic damping compositions are tested for comparison with a sample formed in a manner similar to the samples of Example 1. The samples are tested using the testing method described above with the exception that the test panel is suspended instead of placing it on the foam. Three different samples of QuietGlue® formulations that were acquired over a period of 2 years between 2006 and 2008 are tested. QuietGlue® is commercially available from Quiet Solution of Sunnyvale, Calif. In addition, GREEN GLUE acquired August 2008, available from Green Glue Company of West Fargo, N. Dak., is tested. As illustrated in Table 8, each of the commercially available compositions has a Mode 1 Damping Parameter 0.38 or less. In addition, the samples exhibit low Mode 2 Damping Parameters and low Mode 3 Damping Parameters. In contrast, the sample formed in a manner similar to the samples of Example 1 exhibits a Mode 1 Damping Parameter of at least 0.62 and a Mode 2 Damping Parameter of at least 0.42, far exceeding the damping parameters of the commercially available compositions. In particular, a Damping Performance, defined as the percent increase in damping parameter relative to the GREEN GLUE product as of August 2008, is at least 20% for Mode 1 and Mode 2, such as at least 30%, at least 40%, or even at least 50%.

TABLE 8

| 55     | Mode Damping for Commercial Products |                             |                            |                   |
|--------|--------------------------------------|-----------------------------|----------------------------|-------------------|
|        | Mode Damping                         |                             |                            |                   |
|        | QuietGlue ® (First Sample)           | QuietGlue ® (Second Sample) | QuietGlue ® (Third Sample) | Green Glue Sample |
| Mode 1 | 0.04                                 | 0.12                        | 0.09                       | 0.38 0.62         |
| Mode 2 | 0.09                                 | 0.21                        | 0.18                       | 0.28 0.42         |
| Mode 3 | 0.11                                 | 0.24                        | 0.21                       | 0.31 0.34         |

**13**  
Example 5

Samples are prepared using the Formulation #3 of Example 1 with the addition of EPDM particles of 20 mesh size (<841 microns). The EPDM particles are added in amounts of 3%, 7%, 11%, or 16% by weight.

TABLE 9

| Acoustic Damping for Sample Compositions |      |      |      |      |      |
|------------------------------------------|------|------|------|------|------|
| Mode Damping                             |      |      |      |      |      |
| No Particles                             | 3%   | 7%   | 11%  | 16%  |      |
| Mode 1                                   | 0.54 | 0.49 | 0.48 | 0.49 | 0.40 |
| Mode 2                                   | 0.37 | 0.34 | 0.33 | 0.34 | 0.31 |
| Mode 3                                   | 0.35 | 0.31 | 0.29 | 0.29 | 0.31 |

As illustrated in Table 9, the Mode 1 Damping Parameter decreases slightly with increasing EPDM particle content.

## Example 6

An acoustic damping composition is formed using the Formulation #3 of Example 1 and EPDM particles of 40 mesh size (<420 microns). As illustrated in Table 10, the Mode 1 damping parameter drops less significantly with increasing amounts of EPDM particles, when using EPDM particles of a smaller size than exemplified by the samples of Example 4. (With increasing amounts).

TABLE 10

| Acoustic Damping for Sample Compositions |      |      |      |
|------------------------------------------|------|------|------|
| Mode Damping                             |      |      |      |
| No Particles                             | 7%   | 11%  |      |
| Mode 1                                   | 0.54 | 0.51 | 0.50 |
| Mode 2                                   | 0.37 | 0.38 | 0.34 |
| Mode 3                                   | 0.35 | 0.31 | 0.31 |

## Example 7

An acoustic damping composition is prepared in accordance with Formulation #3 of Example 1 with the addition of polybutylene particles having an average particle size of 60 mesh (<250 microns). In contrast to the samples of Examples 5 and 6, the acoustic damping represented by the Mode 1 Damping Parameter increases, exhibiting a maximum around 3%, as illustrated in Table 11. In addition, the Mode 2 Damping Parameter increases with increasing content of the polybutylene particles.

TABLE 11

| Acoustic Damping of Sample Compositions |      |      |      |
|-----------------------------------------|------|------|------|
| Mode Damping                            |      |      |      |
| No Particles                            | 3%   | 7%   |      |
| Mode 1                                  | 0.54 | 0.61 | 0.55 |
| Mode 2                                  | 0.37 | 0.38 | 0.39 |
| Mode 3                                  | 0.35 | 0.33 | 0.33 |

**14**  
TABLE 12

|        | Acoustic Damping of Sample Compositions |              |                        |              |                      |
|--------|-----------------------------------------|--------------|------------------------|--------------|----------------------|
|        | Mode Damping                            |              |                        |              |                      |
|        | No Particles                            | 20 Mesh EPDM | 30 Mesh Natural Rubber | 40 Mesh EPDM | 60 Mesh Butyl Rubber |
| Mode 1 | 0.54                                    | 0.48         | 0.55                   | 0.51         | 0.55                 |
| Mode 2 | 0.37                                    | 0.33         | 0.30                   | 0.38         | 0.39                 |
| Mode 3 | 0.35                                    | 0.29         | 0.27                   | 0.31         | 0.33                 |

Table 12 illustrates the Mode Damping Parameters for each of the particle types when included in a sample at 7%, based on the Formulation #3 of Example 1. As illustrated, both the 30 mesh natural rubber and 60 mesh polybutylene exhibit improvements in Mode 1 Damping Parameter over the formulations that include no rubber. Further, the 60 mesh polybutylene sample exhibits an increase in the Mode 2 Damping Parameter.

In a first embodiment, an acoustic damping composition includes a binder resin including an addition polymer having a carboxylic functional group, a urethane component, and first elastomeric particles. In an example of the first embodiment, the first elastomeric particles have a modulus of elasticity of not greater than 20 MPa, such as in a range of 0.1 MPa to 20 MPa, or in a range of 0.1 MPa to 10 MPa. In another example, the composition includes 0.1 wt % to 50 wt % of the first elastomeric particles, such as 0.1 wt % to 25 wt % of the first elastomeric particles, or 3.0 wt % to 12 wt % of the first elastomeric particles.

In a further example of the first embodiment, the average particle size of the first elastomeric particles is not greater than 850 micrometers, such as not greater than 600 micrometers, not greater than 450 micrometers, or not greater than 250 micrometers. The average particle size may be at least 1 micrometer.

In an additional example of the first embodiment, the elastomeric particles include a polyolefin rubber, such as polybutylene. In another example, the elastomeric particles include a diene elastomer, such as ethylene propylene diene elastomer. In a further example, the elastomeric particles include a silicone rubber.

In another example of the first embodiment, the acoustic damping composition also includes second elastomeric particles having an average particle size of at least 580 micrometers. The second elastomeric particles have a particle size greater than the first elastomeric particles. For example, the second elastomeric particles have an average particle size of at least 840 micrometers. The composition may include 0.1 wt % to 7 wt % of the second elastomeric particles, such as 0.5 wt % to 5 wt % of the second elastomeric particles.

The acoustic damping composition of the first embodiment may have a Mode 1 Damping Parameter of at least 0.45, such as at least 0.5, at least 0.55, or even at least 0.6. The acoustic damping composition may have a Mode 2 Damping Parameter of at least 0.27, such as at least 0.30, or at least 0.32. The acoustic damping composition may have a Mode 3 Damping Parameter of at least 0.27, such as at least 0.31. The acoustic damping composition may have a Mode 1 Damping Performance of at least 20% or a Mode 2 Damping Performance of at least 20%.

In a further example of the first embodiment, the binder resin and the urethane component are included in a water-based emulsion.

## 15

In a second embodiment, a construction panel includes first and second rigid panels and an acoustic damping composition disposed between the first and second rigid panels. The acoustic damping composition includes a urethane component, elastomeric particles, and a binder resin including an addition polymer having a carboxylic functional group. In an example of the second embodiment, the elastomeric particles have a modulus of elasticity of not greater than 20 MPa. In another example, the acoustic damping composition has a Mode 1 Damping Parameter of at least 0.45.

In a third embodiment a method of preparing a construction panel includes applying an acoustic damping composition to a first major surface of a first rigid panel. The acoustic damping composition includes a urethane component, elastomeric particles, and a binder resin including an addition polymer having a carboxylic functional group. The method further includes contacting a first major surface of a second panel to the acoustic damping composition. In an example of the third embodiment, the elastomeric particles have a modulus of elasticity of not greater than 20 MPa. In another example, the acoustic damping composition has a Mode 1 Damping Parameter of at least 0.45.

In a fourth embodiment, an acoustic damping composition includes a binder resin and first elastomeric particles. The binder resin includes an addition polymer having a carboxylic functional group. The binder resin has a glass transition temperature of not greater than  $-25^{\circ}\text{C}$ . In an example of the fourth embodiment, the glass transition temperature is not greater than  $-40^{\circ}\text{C}$ , such as not greater than  $-50^{\circ}\text{C}$ . In a further example of the fourth embodiment, the acoustic damping composition has a haze of at least 30%.

In an additional example of the fourth embodiment, the first elastomeric particles have a modulus of elasticity of not greater than 20 MPa. In another example, the acoustic damping composition includes 0.1 wt % to 50 wt % of the first elastomeric particles. In a further example the average particle size of the first elastomeric particles is not greater than 450 micrometers. In an additional example, the first elastomeric particles include a polyolefin rubber. Alternatively, the first elastomeric particles include a diene elastomer. In a further alternative, the first elastomeric particles include a silicone rubber.

In a further example, the acoustic damping composition further includes second elastomeric particles having an average particle size of at least 580 micrometers. The second elastomeric particles have a particle size greater than the first elastomeric particles.

In another example, the acoustic damping composition has a Mode 1 Damping Parameter of at least 0.45. In an additional example, the acoustic damping composition has a Mode 2 Damping Parameter of at least 0.27. In a further example, the acoustic damping composition has a Mode 3 Damping Parameter of at least 0.27.

In an additional example, the acoustic damping composition further includes a urethane component. For example, the binder resin and the urethane component can be included in a water-based emulsion.

Note that not all of the activities described above in the general description or the examples are required, that a portion of a specific activity may not be required, and that one or more further activities may be performed in addition to those described. Still further, the order in which activities are listed are not necessarily the order in which they are performed.

## 16

In the foregoing specification, the concepts have been described with reference to specific embodiments. However, one of ordinary skill in the art appreciates that various modifications and changes can be made without departing from the scope of the invention as set forth in the claims below. Accordingly, the specification and figures are to be regarded in an illustrative rather than a restrictive sense, and all such modifications are intended to be included within the scope of invention.

As used herein, the terms "comprises," "comprising," "includes," "including," "has," "having" or any other variation thereof, are intended to cover a non-exclusive inclusion. For example, a process, method, article, or apparatus that comprises a list of features is not necessarily limited only to those features but may include other features not expressly listed or inherent to such process, method, article, or apparatus. Further, unless expressly stated to the contrary, "or" refers to an inclusive-or and not to an exclusive-or. For example, a condition A or B is satisfied by any one of the following: A is true (or present) and B is false (or not present), A is false (or not present) and B is true (or present), and both A and B are true (or present).

Also, the use of "a" or "an" are employed to describe elements and components described herein. This is done merely for convenience and to give a general sense of the scope of the invention. This description should be read to include one or at least one and the singular also includes the plural unless it is obvious that it is meant otherwise.

Benefits, other advantages, and solutions to problems have been described above with regard to specific embodiments. However, the benefits, advantages, solutions to problems, and any feature(s) that may cause any benefit, advantage, or solution to occur or become more pronounced are not to be construed as a critical, required, or essential feature of any or all the claims.

After reading the specification, skilled artisans will appreciate that certain features are, for clarity, described herein in the context of separate embodiments, may also be provided in combination in a single embodiment. Conversely, various features that are, for brevity, described in the context of a single embodiment, may also be provided separately or in any subcombination. Further, references to values stated in ranges include each and every value within that range.

45  
What is claimed is:

1. An acoustic damping composition comprising:  
a water-based emulsion comprising:

50  
a binder resin including an addition polymer having a carboxylic functional group;  
a modifying resin immiscible with the binder resin, the modifying resin comprising a urethane component; and  
a first set of elastomeric particles that decrease the deformability of the acoustic damping composition relative to a same acoustic damping composition absent the first set of elastomeric particles, wherein, when the acoustic damping composition is deployed and dried, the acoustic damping composition has a Mode 1 Damping Parameter of at least 0.45.

60  
2. The acoustic damping composition of claim 1, wherein the binder resin has a glass transition temperature not greater than  $-40^{\circ}\text{C}$ .

65  
3. The acoustic damping composition of claim 1, wherein the first set of elastomeric particles have a modulus of elasticity of not greater than 20 MPa.

## 17

4. The acoustic damping composition of claim 1, comprising 0.1 wt % to 50 wt % of the first set of elastomeric particles.

5. The acoustic damping composition of claim 1, wherein the average particle size of the first set of elastomeric particles is not greater than 850 micrometers.

6. The acoustic damping composition of claim 5, further comprising a second set of elastomeric particles, wherein an average particle size of the second set of elastomeric particles is greater than an average particle size of the first set 10 of elastomeric particles.

7. The acoustic damping composition of claim 6, wherein the second set of elastomeric particles has a different composition than the first set of elastomeric particles.

8. The acoustic damping composition of claim 1, wherein the first set of elastomeric particles includes a polyolefin 15 rubber.

9. The acoustic damping composition of claim 1, wherein the first set of elastomeric particles includes a diene elastomer.

10. The acoustic damping composition of claim 1, wherein the first set of elastomeric particles include a silicone rubber.

11. The acoustic damping composition of claim 1, wherein, when deployed and dried, the acoustic damping composition has a Mode 2 Damping Parameter of at least 0.27.

12. The acoustic damping composition of claim 1, wherein, when deployed and dried, the acoustic damping composition has a Mode 3 Damping Parameter of at least 0.27.

13. The acoustic damping composition of claim 1, wherein, when the acoustic damping composition is deployed and dried, the binder resin, the modifying resin, and the first elastomeric particles each form a different 35 phase.

14. The acoustic damping composition of claim 1, wherein the average particle size of the first elastomeric particles is not greater than 450 micrometers.

15. The acoustic damping composition of claim 1, 40 wherein the water-based emulsion has a solids content of at least 40%.

16. The acoustic damping composition of claim 1, wherein the water-based emulsion has a solids content greater than 60%.

17. The acoustic damping composition of claim 1, 45 wherein, when the acoustic damping composition is

## 18

deployed and dried, the acoustic damping composition has a Mode 1 Damping Parameter of at least 0.5, a Mode 2 Damping Parameter of at least 0.3, and a Mode 3 Damping Parameter of at least 0.27.

18. A construction panel comprising:  
first and second panels; and  
an acoustic damping composition disposed between the first and second panels, the acoustic damping composition comprising:  
a binder resin including an addition polymer having a carboxylic functional group,  
a modifying resin comprising a urethane component, and  
a first set of elastomeric particles,  
wherein the first set elastomeric particles form a separate phase from the rest of the acoustic damping composition; decrease the deformability of the acoustic damping composition relative to a same acoustic damping composition absent the first set of elastomeric particles; and lodge between the first and second panels at pinch points, and  
wherein the acoustic damping composition has a Mode 1 Damping Parameter of at least 0.45.

19. The construction panel of claim 18, wherein the first set of elastomeric particles have a modulus of elasticity of not greater than 20 MPa.

20. An acoustic damping composition layer comprising:  
an acoustic damping composition dried as a film comprising:  
a binder resin forming a first phase, the binder resin including an addition polymer having a carboxylic functional group; and  
a modifying resin forming a second phase separate from the first phase, the modifying resin including a urethane component; and  
a first set of elastomeric particles forming a third phase separate from the first and second phases,  
wherein the first set of elastomeric particles decrease the deformability of the acoustic damping composition layer relative to a same acoustic damping composition layer absent the first set of elastomeric particles, and  
wherein, when the acoustic damping composition is dried as a film, the acoustic damping composition layer has a haze value as measured by ASTM D1003 (method B) of at least 30%.

\* \* \* \* \*